

## UNITED STATES PATENT OFFICE

AUGUST ERNST, OF JOHNSTOWN, NEW YORK

## METHOD OF TANNING CHAMOIS, BUCKSKINS, OR OTHER LEATHER

No Drawing.

Application filed May 8, 1928. Serial No. 276,199.

This invention relates to tanning fur skins, such as chamois, buckskins or the like and has for its object to provide a method whereby an easily washable strong leather that can

be dyed is produced.

This method consists in the following:

After the skins are limed, bated and pickled in the usual manner they are placed in a revolving drum containing formaldehyde in which they are treated for a period of about three-quarters of an hour. Thereupon sod oil or other degras such as Moellen degras dissolved in soap and soda is added to the formaldehyde bath and the treatment of the skins therein continued until the same become tanned. The skins are removed, washed, dried, and scoured.

For clarity in this specification the following definitions of the terms used above are given.

Degras may be defined as any and all greases extracted from oil tanned skins.

Moellen degras may be defined as the "degras" pressed out from skins tanned with sod oil.

Sod oil may be defined as the greases obtained by washing the oil tanned skins in an alkali such as soda or potash solution and treating the fat liquor obtained with sulphuric or other acid to neutralize the same.

What I claim is:

1. A method of tanning leather such as chamois, buckskins or the like, consisting in first liming, bating and pickling the skins, then subjecting them to a treatment under motion in a bath of formaldehyde for about three quarters of an hour, then on adding to said bath degras dissolved in soap and soda the treatment is continued until the skins become tanned, then they are washed, dried and scoured.

2. A method of tanning leather such as chamois, buckskins or the like consisting in first liming, bating and pickling the skins, then subjecting them to a treatment under motion in a bath containing formaldehyde for a period of approximately forty five minutes, then on adding to said bath Moellen degras dissolved in soap and soda, continu-

ing the treatment until the skins become tanned and then washing, drying and scouring said skins.

In testimony whereof I affix my signature.

AUGUST ERNST. 55

60

65

70

75

80

85

90

95

100

**CERTIFICATE OF CORRECTION.**

**Patent No. 1,771,490.**

**Granted July 29, 1930, to**

**AUGUST ERNST**

**It is hereby certified that error appears in the printed specification of the above numbered patent requiring correction as follows: Page 1, line 7, for the word "bated" read bathed, line 25, for "sod" read cod, and in claims 1 and 2, lines 34 and 35, respectively, for "bating" read bathing; and that the said Letters Patent should be read with these corrections therein that the same may conform to the record of the case in the Patent Office.**

**Signed and sealed this 9th day of September, A. D. 1930.**

**(Seal)**

**M. J. Moore,  
Acting Commissioner of Patents.**

CERTIFICATE OF CORRECTION.

Patent No. 1,771,490.

Granted July 29, 1930, to

AUGUST ERNST.

It is hereby certified that Certificate of Correction issued September 9, 1930, was erroneously drawn as to the error in claim 2, and that this Certificate should have read "in claims 1 and 2, lines 34 and 44, respectively, for "bating" read bathing"; that the said Certificate may conform to the records of the office.

Signed and sealed this 30th day of September, A. D. 1930.

(Seal)

M. J. Moore,  
Acting Commissioner of Patents.